

# UNITED STATES PATENT OFFICE.

GREGORY IGOOMNOFF, OF ALATYR, RUSSIA.

## COMPOSITION FOR PAINTING IRON, WOOD, &c.

1,202,847.

Specification of Letters Patent.

Patented Oct. 31, 1916.

No Drawing.

Application filed January 25, 1915. Serial No. 4,367.

To all whom it may concern:

Be it known that I, GREGORY IGOOMNOFF, a subject of the Emperor of Russia, and a resident of Alatyr, Russia, have invented 5 certain new and useful Improvements in Compositions for Painting Iron, Wood, &c., of which the following is a specification.

The green paint ordinarily employed consists largely of high-grade mineral green, 10 which is comparatively very costly, and has a corrosive effect on iron. The improved paint is far cheaper and, at the same time, more brilliant and durable than this mineral green, and has no corrosive effect 15 on iron. For painting iron, wood, etc., both a ground or body paint and a finishing paint are employed, as usual. The composition and the method of preparing both these 20 paints are substantially similar, the difference between them being the addition, to the finishing paint, of certain substances, which are not necessary in the ground or body paint.

In preparing the ground or body paint, 25 sulfate of copper is diluted, together with ordinary hard soap, in water, and the mixture then boiled in a copper or enameled vessel until a homogeneous mixture of sulfate of copper and soap is formed on the surface 30 of the water. The mixture of copper salt and soap thus obtained is carefully separated by decantation from the water and from the various impurities contained in the soap, which impurities settle on the bottom 35 of the kettle during boiling; and after the said mixture has cooled, it is twice washed in pure, cold water. The washed mass is then diluted with ordinary boiled hempseed or other vegetable oil, to which a small 40 quantity of powdered Prussian blue or ultramarine pigment is added. The mass thus prepared is next heated to boiling temperature, and to it, while boiling, are added powdered barium sulfate—*i.e.*, heavy spar,— 45 white lead and chalk, the mass being carefully mixed continuously. After boiling, a sufficient quantity of water is poured into the vessel, and the mass carefully washed in it. The washed mass is carefully rubbed 50 on ordinary rubbing desks or tables such as used in preparing mineral paints, the mass

thus obtained constituting the new ground or body paint. This mass may be diluted, for use, with any desired quantity of boiled 55 vegetable oil.

For preparing the finishing paint, a mixture of sulfate of copper is boiled with hard soap in water until a homogeneous mixture is formed on the surface. This mixture is removed, as before; washed in pure cold 60 water two or more times, and then diluted with boiled hempseed or other vegetable oil, to which a small quantity of Prussian blue or ultramarine pigment and an appropriate 65 quantity of powdered mineral green pigment are added. The mixture obtained is then heated to boiling temperature; and to it, while boiling, are added powdered barium sulfate,—*i.e.*, heavy spar,—white lead and chalk, carefully mixing the mass all the 70 time. After boiling, there is poured into the vessel a sufficient quantity of water, and the boiled mass carefully washed therein. The mass is separated from the water by decantation, or otherwise, and finally is rubbed 75 on rubbing tables. This finishing paint is also diluted for use with any desired quantity of boiled vegetable oil.

The proportions of the materials employed may vary within certain limits; but 80 the following proportions give the best results:

### Ground or body paint.

|                                        | Ounces.           | 85  |
|----------------------------------------|-------------------|-----|
| I. Sulfate of copper                   | 3½                |     |
| Hard soap                              | 9                 |     |
| Boiled hempseed oil                    | 9                 |     |
| Powdered Prussian blue, or ultramarine | 2½                | 90  |
| Powdered heavy spar                    | 25                |     |
| Powdered white lead                    | 9                 |     |
| Chalk                                  | 10                |     |
| II. Sulfate of copper                  | 5                 |     |
| Hard soap                              | 6                 | 95  |
| Boiled hempseed oil                    | 3½                |     |
| Powdered Prussian blue or ultramarine  | 1                 |     |
| Powdered heavy spar                    | 6                 |     |
| Powdered chalk                         | 3                 | 100 |
| Powdered white lead                    | according to      |     |
|                                        | the desired tint. |     |

*Finishing paint.*

|     |                                       | Ounces.                       |                                                                                                                                                                                                |
|-----|---------------------------------------|-------------------------------|------------------------------------------------------------------------------------------------------------------------------------------------------------------------------------------------|
| I.  | Sulfate of copper                     | 8                             | etc., containing sulfate of copper, hard soap, and vegetable oil.                                                                                                                              |
|     | Hard soap                             | 14                            | 25                                                                                                                                                                                             |
| 5   | Boiled hempseed oil                   | 8                             | etc., containing sulfate of copper, hard soap, vegetable oil, and powdered ultramarine.                                                                                                        |
|     | Powdered Prussian blue or ultramarine | $\frac{1}{6}$                 | 3. A composition for painting iron, wood, etc., containing sulfate of copper, hard soap, 30 vegetable oil, powdered ultramarine, barium sulfate, chalk and white lead.                         |
|     | Mineral green pigment                 | $5\frac{1}{2}$                | 4. A composition for painting iron, wood, etc., containing sulfate of copper, hard soap, 35 vegetable oil, powdered ultramarine, barium sulfate, chalk, white lead, and mineral green pigment. |
| 10  | Chalk                                 | 6                             |                                                                                                                                                                                                |
|     | Heavy spar                            | 24                            |                                                                                                                                                                                                |
|     | White lead                            | 24                            |                                                                                                                                                                                                |
| II. | Sulfate of copper                     | 5                             |                                                                                                                                                                                                |
|     | Hard soap                             | 10                            |                                                                                                                                                                                                |
| 15  | Boiled hempseed oil                   | 5                             |                                                                                                                                                                                                |
|     | Powdered Prussian blue or ultramarine | $\frac{1}{6}$                 |                                                                                                                                                                                                |
|     | Powdered mineral green                | $6\frac{1}{2}$                |                                                                                                                                                                                                |
|     | Powdered heavy spar                   | 10                            |                                                                                                                                                                                                |
| 20  | Powdered chalk                        | 3                             |                                                                                                                                                                                                |
|     | Powdered white lead                   | according to<br>desired tint. |                                                                                                                                                                                                |

I claim as my invention:—

1. A composition for painting iron, wood,

In testimony whereof, I have signed my name to this specification in the presence of two subscribing witnesses.

GREGORY IGOOMNOFF.

## Witnesses:

ALEXANDER TSCHERALOFF,  
F. A. LOVIAGUINE.

Copies of this patent may be obtained for five cents each, by addressing the "Commissioner of Patents, Washington, D. C."